

## [54] REINFORCED BONDED ABRASIVE CUP WHEEL

[75] Inventor: James C. Rine, North Tonawanda, N.Y.

[73] Assignee: The Carborundum Company, Niagara Falls, N.Y.

[22] Filed: Apr. 8, 1974

[21] Appl. No.: 458,969

[52] U.S. Cl..... 51/209 R; 51/206 NF

[51] Int. Cl..... B24d 7/04

[58] Field of Search..... 51/206 NF, 209 R; 161/DIG. 4

## [56] References Cited

## UNITED STATES PATENTS

- |           |         |                    |            |
|-----------|---------|--------------------|------------|
| 2,949,698 | 8/1960  | Downey et al.....  | 161/DIG. 4 |
| 3,141,271 | 7/1964  | Fischer et al..... | 51/206 NF  |
| 3,431,687 | 3/1969  | Fischer et al..... | 51/206 NF  |
| 3,540,163 | 11/1970 | Shoemaker .....    | 51/209 R   |
| 3,746,266 | 7/1973  | Knox et al.....    | 51/206 NF  |

## FOREIGN PATENTS OR APPLICATIONS

- |         |        |            |           |
|---------|--------|------------|-----------|
| 580,394 | 8/1958 | Italy..... | 51/206 NF |
|---------|--------|------------|-----------|

Primary Examiner—Al Lawrence Smith

Assistant Examiner—K. J. Ramsey

Attorney, Agent, or Firm—David E. Dougherty;

Raymond W. Green

## [57] ABSTRACT

Bonded abrasive flaring cup wheels, e.g., "Type 11" grinding wheels, are reinforced in the rim portion of the wheel with a substantially flat annular reinforcing strip, typically formed of open mesh woven glass fiber. The annular reinforcing strips are typically formed to a diameter greater than that which will ultimately be required in the grinding wheel and cut at one location in order to allow placement over the diverging frustoconical male mold member used to produce the flaring cup configuration. The ends of the glass fiber reinforcing strip are then overlapped within the mold as the resin coated abrasive grain is being added within the mold cavity. The result is a reinforced bonded abrasive cup wheel having substantially greater strength after having been damaged than the prior art bonded abrasive cup wheel.

12 Claims, 3 Drawing Figures



PATENTED JUL 29 1975

3,896,593

SHEET

1



FIG. I



FIG. 2



FIG. 3

## REINFORCED BONDED ABRASIVE CUP WHEEL

## BACKGROUND OF THE INVENTION

This invention relates to reinforced bonded abrasive cup wheel. More particularly, this invention relates to reinforced bonded abrasive grinding wheels having a back portion and an annular diverging rim portion, the diverging rim portion being integrally formed with the back portion; the diverging rim portion having a diverging frusto-conical inner surface, the smaller diameter of the diverging frusto-conical inner surface being adjacent the back portion of the grinding wheel. This type of wheel is known in the industry as a "flaring cup wheel," and a typical configuration has been given the designation "Type 11" wheel in the United States by the Grinding Wheel Institute. See *American National Standard Safety Code For The Use, Care And Protection Of Abrasive Wheels*, published 1970 by the American National Standard Institute, Inc., the disclosure of which is incorporated by reference. The Type 11 wheel is to be distinguished from the Type 6 straight cup wheel, wherein the rim portion is a non-diverging annulus.

Flaring cup wheels are usually formed in an upright position, with the female mold member, which has the size and shape desired for the outer surface of the annular diverging rim portion of the wheel and for the face of the back portion adjoining the outer surface of the annular diverging rim portion of the wheel, being positioned under and around the wheel which is to be formed. This is done for manufacturing convenience, for example the ability to place within the female mold member, prior to the placement of any bonding material or abrasive grain, a backing plate. This results in the male mold member, which has the size and shape desired for the inner surface of the annular diverging surface of the annular diverging rim portion of the bonded abrasive grinding wheel and for the face of the back portion adjoining the inner surface of the annular diverging rim portion of the wheel, being placed over the initial quantity of abrasive grain and bonding material, prior to building up the annular rim portion of the wheel. The use of substantially flat annular reinforcing strips or discs, such as open mesh woven glass fiber, containing openings of the size between about 2 and about 3 millimeters between the woven filaments of the woven glass fiber, as reinforcements for other types of grinding wheels is conventional. Such reinforcements could be used in the flaring cup wheel without restriction, only prior to the placement of the male mold member within the female mold member. Thus, the back portion of the flaring cup wheel can contain as many substantially flat annular reinforcing strips as may be desired for strength purposes. Once the male mold member has been placed in position, however, the use of conventional (uncut disc-shaped) substantially flat annular reinforcing strips within the wheel, i.e., within the diverging rim portion of the wheel, is restricted, since the inner diameter of the substantially flat annular reinforcing strips will not fit over the male mold member, unless the inner diameter is at least as large as the maximum (upper) diameter of the male mold member. The result is that if reinforcing strips were to be used at all in the rim portion of a flaring cup wheel, the inner diameter of the reinforcing strips would heretofore have had to be at least as large as the

maximum outer diameter of the male mold member which is used to form the rim of the flaring cup wheel.

## SUMMARY OF THE INVENTION

It is, therefore, an object of the invention to provide a bonded abrasive grinding wheel having a back portion and an annular diverging rim portion, the diverging rim portion being integrally formed with the back portion; the diverging rim portion having a diverging frusto-conical inner surface, the smaller diameter of the diverging frusto-conical inner surface being adjacent the back portion of the grinding wheel; wherein the improvement comprises the provision of at least one substantially flat annular reinforcing strip within the diverging rim portion of the grinding wheel, the annular reinforcing strip being substantially perpendicular to the axis of the frusto-conical inner surface of the diverging rim portion, and the inner diameter of the annular reinforcing strip being less than the maximum diameter of the diverging frusto-conical inner surface of the diverging rim portion of the grinding wheel. Such a bonded abrasive grinding wheel can be produced, in accordance with the present invention, by (1) placing a quantity of abrasive grain coated with uncured resin in a female mold member, the female mold member having the size and shape desired for the outer surface of the annular diverging rim portion of the bonded abrasive grinding wheel and for the face of the back portion of the grinding wheel adjoining the outer surface of the annular diverging rim portion of the grinding wheel, the quantity of resin coated abrasive grain being sufficient to fill the female mold member to the level corresponding to the smaller diameter of the diverging frusto-conical inner surface of the diverging rim portion of the bonded abrasive grinding wheel; (2) placing within the female mold member a male mold member, over the quantity of resin coated abrasive grain within the female mold member, the male mold member having the size and shape desired for the inner surface of the annular diverging surface of the annular diverging rim portion of the grinding wheel and for the face of the back portion of the grinding wheel adjoining the inner surface of the annular diverging rim portion of the bonded abrasive grinding wheel, for forming a cavity corresponding to the annular diverging rim portion between the female mold member and the male mold member; (3) placing additional abrasive grain coated with uncured resin in the cavity between the female mold member and the male mold member, while (4) periodically inserting within the cavity between the female mold member and the male mold member, the substantially flat annular reinforcing strips, the annular reinforcing strips having, after placement, an inner diameter less than the maximum diameter of the diverging frusto-conical inner surface of the diverging rim portion of the grinding wheel, and being placed substantially perpendicular to the axis of the male mold member; and (5) compressing and curing the resin coating of the abrasive grain, for forming an integrally bonded abrasive grinding wheel.

## BRIEF DESCRIPTION OF THE DRAWINGS

FIG. 1 is a vertical sectional view of a reinforced bonded abrasive grinding wheel in accordance with the present invention.

FIG. 2 is a broken away section of the wheel illustrated in FIG. 1, taken along line 2-2 of FIG. 1.

FIG. 3 illustrates the orientation of the grinding wheel with respect to the male and female mold members during the production of the grinding wheel.

#### DETAILED DISCLOSURE

Referring now to FIG. 1, there is illustrated a vertical cross-section of a reinforced bonded abrasive grinding wheel in accordance with the present invention. The wheel comprises a back portion 11 and an annular diverging rim portion 12, the diverging rim portion 12 being integrally formed with the back portion 11. The diverging rim portion 12 has a diverging frusto-conical inner surface 13, the smaller diameter 14 of the diverging frusto-conical inner surface 13 being adjacent the back portion 11. The improvement in accordance with the present invention comprises the provision of at least one, and preferably a plurality, of substantially flat annular reinforcing strips 15-17 within the diverging rim portion 12 of the grinding wheel. The phrase "substantially flat annular reinforcing strip" as used herein is generic to both an endless strip or disc, having been cut with only an inner circumference and an outer circumference, and a slit strip or disc, i.e., an annular reinforcing strip which has been provided with a pair of end portions, for example by cutting an endless annular reinforcing strip. If a plurality of annular reinforcing strips 15-17 is used, they are preferably substantially equally axially spaced throughout the annular rim portion 12 of the grinding wheel. If desired, there may be provided one or more additional annular reinforcing strips 18 between the back portion 11 and the rim portion 12, or 19 within the back portion 11 of the grinding wheel. The annular reinforcing strip or strips 15-19 are substantially perpendicular to the axis 21 of the frusto-conical inner surface 13 of the diverging rim portion 12 of the grinding wheel. The inner diameters of the annular reinforcing strips 15-17 within the annular diverging rim portion 12 of the grinding wheel are less than the maximum diameter 22 of the diverging frusto-conical inner surface 13 of the diverging rim portion 12 of the grinding wheel.

In accordance with one embodiment of the present invention, the annular reinforcing strips 15-19 are provided with indentations for engagement with binder material of the grinding wheel. The annular reinforcing strips could also be provided with protruberances for engagement with binder material of the grinding wheel. It is much preferred, however, that the annular reinforcing strips be provided with interstices (i.e., openings) for penetration with binder material of the grinding wheel, as this provides greater reinforcement. It is further preferred, moreover, that the annular reinforcing strip or strips be woven filamentary material, in particular woven filamentary material having interstices formed therein, the interstices being openings between the woven filaments of the woven filamentary material, the openings ranging in size between about 2 and about 3 millimeters. A particularly preferred woven filamentary material for this use is glass fiber, which is commercially available in woven form.

In some cases, it will be feasible to produce the grinding wheel of the invention with the male mold member on the underside, so that the annular reinforcing strips are endless discs, which can be placed over the male mold member as the annular diverging rim portion 12 of the grinding wheel is being built up. In other cases, it will be feasible to utilize segmented male mold mem-

bers, so that only a portion of the male mold member is inserted prior to the placement of the first annular reinforcing strip within the diverging rim portion 12 of the grinding wheel. In such a case, the annular reinforcing strips need not be cut or overlapped within the annular diverging rim portion 12 of the grinding wheel. In the more common situation, however, it will be preferred to build up the grinding wheel with the female mold member underneath the grinding wheel, a single piece male mold member being used. This may be desirable, for example, if a backing plate is placed within the grinding wheel within the female mold member, prior to placing any resin coated abrasive grain in the female mold member. In such a case, the annular reinforcing strip or strips are provided with a pair of end portions 25 and 26 (see FIG. 2), suitably by cutting an oversize annular reinforcing strip (for example, along the radius of the annular reinforcing strip). By "oversize" it is meant that the annular strips will have greater inner and outer diameters, prior to cutting, than that of the annular rim portion 12 of the grinding wheel. The end portions of each annular reinforcing strip are then disposed within the annular diverging rim portion 12 of the grinding wheel in overlapping relationship, as illustrated in FIG. 2, wherein the numeral 27 designates the overlapping section of end portions 25 and 26. It is preferred that the overlapped end portions of the annular reinforcing strip or strips are overlapped an amount equal in distance to at least about one width of the annular reinforcing strip. As used herein, the "width" of the annular reinforcing strip is the difference between a radius of the outside diameter and a radius of the inside diameter of the annular reinforcing strip.

In addition to providing a plurality of annular reinforcing strips substantially equally axially spaced throughout the annular rim portion of the grinding wheel, it is preferred that the annular reinforcing strips be spaced at axial intervals at least as close as one-half inch between the annular reinforcing strips.

The preferred process for producing a bonded abrasive grinding wheel in accordance with the present invention will now be described, with reference to FIG. 3. If desired, a backing plate 23 is first placed within the female mold member 29. The backing plate 23 may be provided with protruding portions 30 for engagement within the back portion 11 of the grinding wheel, and also with threaded portion 31 for engagement with a grinding machine for use of the wheel.

Next, or first if no backing plate is to be used, a quantity of abrasive grain coated with uncured resin is placed in the female mold member 29, the female mold member 29 having the size and shape desired for the outer surface 32 of annular diverging rim portion 12 and for the face 33 of the back portion 11 of the grinding wheel adjoining the outer surface 32 of the annular diverging rim portion 12 of the grinding wheel. The quantity of resin coated abrasive grain provided at this point is sufficient to fill the female mold member to the level corresponding to the smaller diameter 14 of the diverging frusto-conical inner surface 13 of the diverging rim portion 12 of the bonded abrasive grinding wheel.

At this point, it is preferred to place one additional annular reinforcing strip 18 within the female mold member 29, over the quantity of resin coated abrasive grain filling the female mold member 29 to the level corresponding to the smaller diameter 14 of the diver-

ing frusto-conical inner surface 13 of diverging rim portion 12 of the grinding wheel.

Next there is placed within the female mold member 29 a male mold member 35, over the quantity of resin coated abrasive grain within the female mold member 29. The male mold member has the size and shape desired for the inner surface 13 of the diverging rim portion 12 of the grinding wheel, and of the face 36 of the back portion 11 of the grinding wheel adjoining the inner surface 13 of the annular diverging rim portion 12 of the grinding wheel. There is thus formed a cavity corresponding to the annular diverging rim portion 12 of the grinding wheel, between the female mold member 29 and the male mold member 35.

Additional abrasive grain coated with uncured resin is then placed in the cavity between the female mold member 29 and the male mold member 35, while periodically inserting, within the cavity between the female mold member 29 and the male mold member 35, the substantially flat annular reinforcing strips 15-17, the annular reinforcing strips 15-17 having, after placement, an inner diameter less than the maximum diameter 22 of the diverging frusto-conical inner surface 13 of the diverging rim portion 12 of the grinding wheel. The annular reinforcing strips are also placed substantially perpendicular to the axis 21 of the male mold member which is, of course, the same as the axis 21 of the frusto-conical inner surface 13 of the diverging rim portion 12 of the grinding wheel after the grinding wheel is completed.

The resin coating of the abrasive grain is then compressed and removed from the mold, and cured in a conventional manner such as by placing the grinding wheel into a kiln. Any conventional resin can be used, however, phenolic resins (i.e., phenol-aldehyde resins) are usually preferred.

It is also preferred that the annular reinforcing strips include end portions, the end portions being disposed in overlapping relationship, as illustrated in FIG. 2.

If desired, at least one additional annular reinforcing strip 19 can be placed within the female mold member 29 within the resin coated abrasive grain filling the female mold member 29 to the level corresponding to the smaller diameter 34 of the diverging frusto-conical inner surface 13 of the diverging rim portion 12 of the grinding wheel. Such additional annular reinforcing strips will usually not be necessary however, if the backing plate 23 including protruding portions 30 is utilized.

The invention will now be illustrated with an example.

#### EXAMPLE

A series of Type 11 bonded abrasive grinding wheels having the cross-section illustrated in FIG. 1 were produced with zero, three or four annular reinforcing strips 15-18. The larger outer diameter (dimension "D" as identified at page 10 of the above publication of the American National Standard Institute was 6 inches. The smaller outer diameter (dimension "J") was 4 $\frac{1}{4}$  inches. The thickness ("T") was 2 inches. The width of the rim face ("W") was 1 $\frac{1}{4}$  inches, and the thickness of the back portion ("E") was  $\frac{3}{8}$  inch. The smaller inner diameter of the annular rim portion 12 ("K") was 2 $\frac{1}{2}$  inches. The discs were provided with a reinforcing backing plate 23, having a  $\frac{5}{8}$  inch thread, 11 threads per inch. The wheels were constructed of

phenolic resin bonded aluminum oxide grain. The only differences between the wheels were the number and locations of annular reinforcing strips 15-18 provided in the wheels. In all cases, the reinforcing strips were woven glass fiber having a basket weave, the larger openings between the woven filaments ranging in size between about 2 and about 3 millimeters, square. In all cases, for reinforced wheels one glass fiber reinforcing strip 18 was placed between the back portion 11 and the annular rim portion 12 of the grinding wheel. For those wheels containing four reinforcing strips, second, third and fourth strips were placed at substantially equally spaced intervals throughout the annular rim portion of the grinding wheel, at axial intervals slightly less than  $\frac{1}{2}$  inch between the annular reinforcing strips. The grinding wheels containing three annular reinforcing strips had various configurations for the second and third strips.

Various discs produced as indicated above were subjected to speed tests, in which the grinding wheels were tested for ultimate speed in surface feet/minute attainable prior to fracture. The grinding wheels in some cases were subjected to impact loads ranging up to 74 ft. pounds, in various locations relative to the grinding wheel. The results of these tests are set forth in Table 1. In Table 1, under the heading "TYPE OF IMPACT," the letter "A" indicates a 1-inch line impact parallel to the axis of the grinding wheel, on the grinding face (the 1 $\frac{1}{4}$  inch wide annular face of the diverging annular rim portion 12 of the grinding wheel). The letter "B" indicates an impact perpendicular to the axis of the grinding wheel, concentrated at the maximum diameter at the edge of the rim portion 12. The letter "C" indicates a line impact perpendicular to the axis of the grinding wheel, spread over about 1 inch of the outer surface 32 of the annular rim portion 12. The ultimate speeds obtainable after receiving the impacts indicated are set out in Table 1.

TABLE 1

| IMPACT<br>(FOOT-POUNDS) | TYPE OF<br>IMPACT | NUMBER OF<br>REINFORCING<br>STRIPS | ULTIMATE<br>SPEED (SFPM) |
|-------------------------|-------------------|------------------------------------|--------------------------|
| 45                      | NONE              | —                                  | 19,800                   |
| 24                      | A                 | 0                                  | 7,050                    |
| 34                      | A                 | 0                                  | 9,500                    |
| 54                      | A                 | 0                                  | 18,500                   |
| 44                      | A                 | 3                                  | 14,700                   |
| 54                      | A                 | 3                                  | 14,870                   |
| 64                      | A                 | 3                                  | 14,300                   |
| 74                      | A                 | 3                                  | 14,000                   |
| 50                      | NONE              | —                                  | 12,100                   |
| 44                      | A                 | 3                                  | 12,100                   |
| 54                      | A                 | 3                                  | 12,100                   |
| 64                      | A                 | 3                                  | 18,000                   |
| 74                      | A                 | 3                                  | 15,400                   |
| 55                      | NONE              | —                                  | 14,600                   |
| 44                      | A                 | 4                                  | 14,100                   |
| 54                      | A                 | 4                                  | 14,800                   |
| 64                      | A                 | 4                                  | 14,700                   |
| 74                      | A                 | 4                                  | 15,000                   |
| 3 $\times$ 54 (1)       | A                 | 4                                  | 14,800                   |
| 3 $\times$ 54 (2)       | A                 | 4                                  | 14,900                   |
| 3 $\times$ 74 (1)       | A                 | 4                                  | 16,900                   |
| 54                      | B                 | 4                                  | 16,200                   |
| 54                      | C                 | 4                                  | 16,200                   |

60 (1) Three impacts in same location.

(2) Three impacts in different locations.

In Table 1, each ultimate speed shown is the average of three trials, of identical wheels which had been subjected to identical impact testing.

65 From the above, it can be concluded that the inclusion of substantially flat annular reinforcing strips within the diverging rim portion of the grinding wheel

represents a substantial improvement in ultimate speed to which the grinding wheel can be subjected, after having received an impact such as might be accidentally sustained during use, which would crack the bonding system of the grinding wheel. Wheels made in accordance with the present invention unexpectedly have no disproportionate weakness at the location at which the glass fiber reinforcing strips are overlapped within the rim portion of the wheel.

I claim:

1. A bonded abrasive grinding wheel having a back portion and an annular diverging rim portion, the diverging rim portion being integrally formed with the back portion; the diverging rim portion having a diverging frusto-conical inner surface, the smaller diameter of the diverging frusto-conical inner surface being adjacent the back portion of the grinding wheel;

wherein the improvement comprises the provision of at least one substantially flat annular reinforcing strip of woven filamentary material having therein interstices for penetration with binder material of the grinding wheel, within the diverging rim portion of the grinding wheel, the annular reinforcing strip being substantially perpendicular to the axis of the frusto-conical inner surface of the diverging rim portion, and the inner diameter of the annular reinforcing strip being less than the maximum diameter of the diverging frusto-conical inner surface of the diverging rim portion of the grinding wheel; wherein the annular reinforcing strip includes a pair of end portions, the end portions being disposed in overlapping relationship.

2. A bonded abrasive grinding wheel according to claim 1, the openings ranging in size between about 2 and about 3 millimeters.

3. A bonded abrasive grinding wheel according to claim 2, wherein the woven filamentary material is glass fiber.

4. A bonded abrasive grinding wheel according to claim 1, wherein the overlapped end portions of the annular reinforcing strip are overlapped an amount equal in distance to at least about one width of the annular reinforcing strip.

5. A bonded abrasive grinding wheel according to claim 1, comprising a plurality of annular reinforcing strips within the diverging rim portion of the grinding wheel.

6. A bonded abrasive grinding wheel according to claim 5, wherein the plurality of annular reinforcing strips are substantially equally axially spaced throughout the annular rim portion of the grinding wheel.

7. A bonded abrasive grinding wheel according to claim 5, wherein the annular reinforcing strips are each woven glass fiber, the strips being provided with openings of a size between about 2 and about 3 millimeters between the woven filaments of the woven glass fiber, and having ends overlapped an equal amount equal to at least about one width of the annular reinforcing strip.

8. A bonded abrasive grinding wheel according to claim 7, wherein the annular reinforcing strips are spaced at axial intervals at least as close as one-half inch between the annular reinforcing strips.

9. A process for producing a bonded abrasive grinding wheel according to claim 1, comprising the steps of

1. placing a quantity of abrasive grain coated with un-

10

5

35

45

50

55

60

65

cured resin in a female mold member, the female mold member having the size and shape desired for the outer surface of the annular diverging rim portion of the bonded abrasive grinding wheel and for the face of the back portion of the grinding wheel adjoining the outer surface of the annular diverging rim portion of the grinding wheel, the quantity of resin coated abrasive grain being sufficient to fill the female mold member to the level corresponding to the smaller diameter of the diverging frusto-conical inner surface of the diverging rim portion of the bonded abrasive grinding wheel;

2. placing within the female mold member a male mold member, over the quantity of resin coated abrasive grain within the female mold member, the male mold member having the size and shape desired for the inner surface of the annular diverging surface of the annular diverging rim portion of the bonded abrasive grinding wheel and for the face of the back portion of the grinding wheel adjoining the inner surface of the annular diverging rim portion of the bonded abrasive grinding wheel, for forming a cavity corresponding to the annular diverging rim portion between the female mold member and the male mold member;

3. placing additional abrasive grain coated with uncured resin in the cavity between the female mold member and the male mold member, while

4. periodically inserting, with the cavity between the female mold member and the male mold member, the substantially flat annular reinforcing strips, the annular reinforcing strips having, after placement, an inner diameter less than the maximum diameter of the diverging frusto-conical inner surface of the diverging rim portion of the grinding wheel, and being placed substantially perpendicular to the axis of the male mold member; wherein the annular reinforcing strips include end portions, the end portions being disposed in overlapping relationship; and

5. compressing and curing the resin coating of the abrasive grain, for forming an integrally bonded abrasive grinding wheel.

10. A process according to claim 9, comprising in addition placing within the female mold member an additional substantially flat annular reinforcing strip, over the quantity of resin coated abrasive grain filling the female mold member to the level corresponding to the smaller diameter of the diverging frusto-conical inner surface of the diverging rim portion of the grinding wheel, prior to placement of the male mold member within the female mold member.

11. A process according to claim 9, comprising in addition placing at least one additional annular reinforcing strip within the female mold member within the resin coated abrasive grain filling the female mold member to the level corresponding to the smaller diameter of the diverging frusto-conical inner surface of the diverging rim portion of the bonded abrasive grinding wheel.

12. A process according to claim 9, comprising in addition placing a backing plate within the female mold member, prior to placing any resin coated abrasive grain in the female mold member.

\* \* \* \* \*